

## UNITED STATES PATENT OFFICE

1,973,302

## ALLOY

Robert J. Wiseman, Passaic, and Benjamin B. Reinitz, Paterson, N. J., assignors to The Okonite-Callender Cable Company, Incorporated, Paterson, N. J., a corporation of New Jersey

No Drawing. Application September 14, 1933,  
Serial No. 689,428

## 2 Claims. (Cl. 75-1)

Our invention is directed to an alloy of lead and has for one of its objects the provision of an alloy which is particularly well adapted for the sheaths of electric power cables, our improved alloy possessing characteristics which are very desirable in such use.

The quality of impregnated paper cables for the transmission and distribution of electric power has been greatly improved during the past 10 few years by reason of the quality of the paper and oil used and the manufacturing processes employed. As a result, the number of cable failures due to the insulation has been reduced. On the other hand, an increase in the number 15 of failures assignable to the lead sheath—the protective covering for the insulation—has been noted. This increase in sheath failures is partially due to the higher internal pressures which occur in present day cables as a result of the 20 greater amount of oil employed and partially to the physical characteristics of pure lead. Lead is a comparatively soft, ductile metal, having practically no yield point and consequently, even with moderate stresses, it will stretch. In the 25 case of lead sheath, this means thinning of the lead wall and eventually rupturing of the sheath as it no longer is able to withstand the internal pressures existing in the cable as it heats up due to carrying a power load.

30 The lead alloy of the present invention is strong and tough, but not brittle. Its physical properties, such as tensile strength and elongation, show it to be much superior to ordinary lead, in that its tensile strength is much higher 35 and its elongation lower. Where with ordinary lead the yield point is very low, the yield point of our alloy is only slightly less than its ultimate strength. This is most helpful as it permits of a very much higher internal pressure in 40 a cable without stretching of the sheath. For example, we have noted for the same size sheath and wall thickness an expansion six to eight times as much for ordinary lead as for our alloy.

This is due to the remarkable homogeneity of 45 the mixture and small grain or crystal structure. The usual types of alloys of lead, such as tin and lead or antimony and lead, do not act in a similar manner. In fact, one of the objections to the use of such alloys is the ease of segregation of the tin or antimony before sheathing. This does not occur with the alloy of the present invention. Furthermore, the thorough mixing of the materials of our alloy aids greatly in 50 obtaining a uniform sheath, thereby improving the stability and strength of the sheath in service.

In addition to all of the foregoing, our alloy not only is superior to ordinary lead as a sheath material in service, but is also a superior metal to run on the lead press. The covering of an 55 electric power cable with a sheath is an inter-

mittent operation. As the cable advances through the press die block the plastic metal is forced through the die under extremely high pressure. When the supply or charge of lead is exhausted the "run" is stopped, the press cylinder is refilled and allowed to cool, and then the new charge of metal is forced through the die as before. At the end of each of these "runs" there is always some lead known commercially as a "slug", left in the press, and the surface of this "slug" becomes oxidized in spite of all care exercised to prevent it, so that a homogeneous bond between the fresh charge of metal and the preceding charge is prevented by reason of the presence of this oxide. We have found 75 that the resistance of our alloy to oxidation is very high and hence oxidation of the "slug" to a detrimental extent does not occur, thereby insuring a homogeneous bond between the fresh metal and that of the preceding charge. 80

We also find that our alloy is more easily extruded than other alloys of lead, permitting a rate of extrusion almost the equal of pure lead. We have noted also that due to its higher resistance to oxidation during extrusion our material 85 is clean and free from dross and blisters.

Our alloy furthermore has shown itself to be highly resistant to corrosion, a characteristic which makes it very advantageous for use as a power cable sheath for installation in ducts or for 90 burying directly in the ground.

Our alloy contains lead and a small quantity of antimony and vanadium, and while the proportions of these materials may be varied somewhat, we have found good results when these materials 95 are used in the following range of proportions:

|          |                  |
|----------|------------------|
| Lead     | 98.85% to 99.75% |
| Antimony | .25% to 1%       |
| Vanadium | .005% to .15%    |

100 it being understood that in any event the amount of lead employed is far in excess of the antimony and vanadium.

What we claim is:—

1. An alloy comprising lead, antimony and vanadium in the proportions of:

|          |                  |
|----------|------------------|
| Lead     | 98.85% to 99.75% |
| Antimony | .25% to 1%       |
| Vanadium | .005% to .15%    |

110 2. A lead alloy sheath for electric power cables consisting of lead, antimony and vanadium in the proportions of:

|          |                  |
|----------|------------------|
| Lead     | 98.85% to 99.75% |
| Antimony | .25% to 1%       |
| Vanadium | .005% to .15%    |

ROBERT J. WISEMAN.  
BENJAMIN B. REINITZ. 120